

Patented Nov. 23, 1926.

1,607,994

# UNITED STATES PATENT OFFICE.

CHARLES P. MADSEN, OF NEW YORK, N. Y., ASSIGNOR TO MADSENELL CORPORATION,  
OF NEW YORK, N. Y., A CORPORATION OF NEW YORK.

## MEANS FOR ELECTRODEPOSITING METALS.

No Drawing. Application filed August 4, 1921, Serial No. 489,852. Renewed June 4, 1926.

My present invention relates to the electrodeposition of metals, particularly the "nickel metals", by which I mean metals of the nickel group, particularly nickel, cobalt, and alloys containing substantial amounts of either or of both of these metals. It is an object of the present invention to provide means for electrodepositing such metals in such a form that they will be mechanically perfect, that is, substantially free from pores and pits, and will be annealable as well as ductile and malleable. It is a further object of the present invention to devise means of the character described which will be simple to put into operation and which will permit the production of metal of the character specified within a wider range of working conditions than has heretofore been deemed possible. In other words, it is an object of the present invention to provide a readily workable, commercial process for electrodepositing "nickel metals", the process being so simple and effective as to permit its ready adoption and operation under ordinary factory conditions without elaborate precautions and without a large number of tests and checks to ensure this proper result.

In the accompanying specification I shall set forth several illustrative embodiments of the means of my present invention, it being understood, however, that my invention is not limited to the particular embodiments thereof which are herein described for purposes of illustration only.

Before describing in detail the aforesaid illustrative embodiments of my present invention, it may be desirable to point out briefly certain disadvantages of the prior art relating to the electrodeposition of the "nickel metals."

Electrolytic nickel as ordinarily produced is a brittle, almost friable, material, which cannot be made ductile even by annealing. It is generally understood that this condition is due largely to the presence of hydrogen in the electrolytic nickel. However, nickel made by processes calculated to remove the hydrogen, although initially slightly more malleable than the ordinary electrolytic nickel, becomes less so upon annealing, while both kinds of electrolytic nickel as now made are frequently filled with deep pits, for which no permanent remedy has hitherto been found.

In my copending application, Serial No. 254,793 filed Sept. 19, 1918, entitled Process for the electrodeposition of metals, I have disclosed means for mechanically manipulating the cathode so as to largely, and in many instances, entirely, avoid the formation of pits.

In another copending application, Serial No. 292,793 filed April 26, 1919, entitled Electrodeposition of metals, I have disclosed an improved form of bath by means of which, when the factors of deposition are properly regulated, I may still further minimize the formation of pits and at the same time produce a metal which is annealable.

In still another copending application, Serial No. 388,812 filed June 14, 1920, and entitled Anodes and methods of preparing the same I have disclosed a new type of anode which practically continuously maintains the proper working conditions of my new bath mentioned above, and by means of which I am enabled, in combination with the mechanical manipulation of the cathode described above, to produce pitless "nickel metal" of a high degree of ductility, which metal is at the same time annealable. I have, in fact, under favorable conditions produced such metal by a process which uses only the above bath and anode.

I have discovered new means for accomplishing the same general result of my previously filed applications referred to above by which new means I greatly simplify the process and substantially increase the range of working conditions within which I may operate to obtain pitless, malleable, ductile and annealable "nickel metal". While I may use the new means of my present invention to great advantage in connection with most of the old and well known nickel electrodeposition processes with which I am familiar, my present invention finds particularly successful application in connection with the bath and anode of my two previously filed applications last referred to above.

It has been thought for some time that hydrogen is a factor in causing the formation of pits, but prior to the development of the improvements referred to above, means for the complete removal of hydrogen had not been found, and the mechanism of pit formation has not, until my present in-

vention, been satisfactorily explained. The indications are that another factor in the formations of pits is the presence in the bath of solid foreign particles. These particles 5 are often deposited on the cathode, and, either by catalysis or by the formation of a local cell, or for both reasons, apparently cause the combination of atomic hydrogen into molecular hydrogen which is discharged 10 in a gas stream at each point of the cathode where such a particle has become lodged, thereby preventing the deposition of nickel metal and thus forming a pit. Some of these particles may be in the nature of colloidal or finely divided metallic nickel, or graphite, carbides, or other impurities carried over mechanically from the anode.

I have, moreover, discovered that another 20 class of foreign bodies, which I believe has not hitherto been suspected as being a factor in the formation of pits, is probably another cause of pit formation. This class comprises organic materials in the nature of small particles of dust, spores, bacteria, microscopic 25 seeds, and the like. Most of these organic particles drop in from the air during electrolysis, but many of them are already present in the commercial nickel salts and in the other materials from which the bath is made 30 up. It appears that not only can these organic materials exist in the bath but that they may even propagate and grow there. I have found large growths of funga and other plant life, the exact description of 35 which, however, is unknown, present in nickel baths which have stood idle for as long as several weeks.

That these organic materials comprise one 40 of the factors of pit formation is indicated by the fact that a newly prepared bath generally makes more pits than one which has been in continuous use. Moreover, a bath which has been standing idle for several 45 weeks makes still more pits than either of the baths mentioned above, and in this case the organic material is often clearly visible. Removal of this organic material by filtration or other mechanical means alone is not effective, neither has it been found practical 50 to prevent the transfer of foreign particles from the anode by means of bags, as any bag material fine enough to stop the particles will interfere with the electrolysis.

I have stated above that all, and particularly 55 commercial nickel, salts and other ingredients used in making up a nickel bath, contain organic material. Commercial nickel salts also contain iron and copper, generally in the form of their chlorides and sulphates. I prefer, therefore, as a preliminary step to 60 my new process, to purify the nickel salts or electrolyte made from the same. For this purpose I may use any agent, preferably an oxidizing agent, which will act to remove the 65 organic matter and also the iron and copper

salts from the nickel salts or from the electrolyte containing the same in solution. Where, as is preferred, an oxidizing agent is used for this purpose, I find that there are several oxidizing agents which, while they 70 will remove the organic matter and the iron, will not ordinarily effect the removal of the copper. I have found, however, that the use of chlorine gas as the oxidizing agent will, under certain conditions, produce a new and 75 unexpected result in that this agent not only removes the organic matter and the iron from the bath, but at the same time removes substantially all of the copper.

To carry out this proposed preliminary 80 purifying step, I preferably make up a concentrated nickel salt solution intended to contain, for example, about 240 grams of nickel sulphate and about 20 grams of nickel chloride per liter of bath, by dissolving the salts 85 in only half of the required amount of water, at the same time heating this concentrated solution of nickel salts to keep the same in solution, for which purpose I prefer to heat the concentrated solution to a temperature of 90 from 30° to about 40° C. To the other half of the required water I add an amount of caustic, as sodium, hydrate, somewhat in excess of the chemical equivalent of the free acid and of the iron and copper salts present 95 in the nickel salt solution.

These two solutions are then mixed together and stirred very rapidly. An almost complete and immediate alkalinization of the 100 solution takes place, precipitating very little nickel, while the iron is at once precipitated in the form of a precipitate of gelatinous or colloidal ferrous hydrate, which acts as a reducing agent. Chlorine gas is now bubbled 105 slowly through the mixture while stirring the same, the addition of chlorine gas continuing until the precipitate, as indicated by a sample, is of a light brown color. If the ferrous hydrate has not been oxidized to the point indicated by the light brown color of 110 the precipitate, it will not filter out readily, whereas if the chlorination is carried out much beyond this point, the copper apparently goes into solution again. All of the 115 reasons for this action are not clearly understood. My present theory, however, is that the cupric sulphate present in the bath is converted into the corresponding chloride which, in the presence of the ferrous hydrate initially present in the bath, is reduced to 120 cuprous chloride, with the simultaneous oxidation of the ferrous hydrate to the ferric condition indicated by the light brown color referred to. The cuprous chloride, being insoluble, is precipitated from the solution 125 while the ferrous hydrate, which has acted as a reducing agent for converting the cupric salt into the cuprous condition and which has thus been converted into the ferric state, settles all the more readily than it otherwise 130

would. It may here be stated that there is generally more than sufficient ferrous hydrate produced by the preliminary neutralizing step than is theoretically needed for reducing the copper from the cupric to the cuprous condition. From this explanation it follows that an excess of chlorine would convert the cuprous chloride into the soluble cupric chloride, a condition to be avoided.

10 The bath thus treated is now filtered and 40 grams of boric acid per litre of bath added. Where the bath is to be used with an anode which is being used as such for the first time, it may be desirable to permit 15 any residual chlorine to remain in the bath, since this residual chlorine is carried by the current to the anode, where it acts to more effectively help to dissolve the same and to break down the outer, difficultly soluble 20 "skin" present on many types of anodes. Otherwise, the residual chlorine may be eliminated by any suitable means, as by boiling the bath.

A bath so prepared will, in combination 25 with my anodes referred to above, produce ductile, pitless and annealable nickel until particles commence to be transferred from the anodes. At this juncture pits may form. Moreover, if the anode-cathode 30 surface ratio is not correct, the "pH" reading may change and cause pits to be formed. Furthermore, after such a bath has been kept standing idle for even comparatively short periods, especially if the bath is warm, 35 pits may be formed on resuming operation of the bath. In such cases re-chlorinating the bath is often effective in preventing further pit formation.

I have, however, discovered that other 40 oxidizing agents besides chlorine are effective in overcoming the pits when they once commence to be formed after the bath has been preliminarily treated with chlorine. Such other oxidizing agents effective in preventing pit formations comprise, for instance, the permanganates and also those salts which, during electrolysis, pass through intermediate stages during which they give off oxygen. An example of these 50 latter salts is manganese sulphate. However, these materials are open to the objection that the by-products of decomposition either make more sludge, which may serve to darken and roughen the deposit and to 55 cause other difficulties, or may add increasing amounts of undesirable soluble salts to the electrolyte.

I have discovered that hydrogen peroxide 60 is even more effective than any of these reagents and is even more effective than chlorine for preventing pit formation after the preliminary oxidation treatment, although hydrogen peroxide may also be used for the preliminary oxidation treatment, although 65 for this purpose it is not so effective for

removing the copper, however efficient it is for precipitating the iron and oxidizing the organic matter present in the bath. Hydrogen peroxide is desirable for use for pit prevention since it does not produce any 70 sludge, nor does it add any undesirable or other soluble salts to the bath. It is also probable that the hydrogen peroxide produces other desirable results in the bath than that of merely oxidizing the organic 75 matter. In fact, this substance appears to act as a perfect cathode depolarizer to prevent the evolution of hydrogen in either atomic or molecular condition at the cathode and thus to prevent the formation of 80 pits.

Under the above conditions the hydrogen, in atomic or molecular condition, decomposes hydrogen peroxide instantly, with the formation of water. It is therefore 85 believed that the presence of hydrogen peroxide in the bath acts as a true cathode depolarizer by combining chemically with both atomic and molecular hydrogen as soon as the same is formed. The hydrogen peroxide thereby acts to remove one of the principal factors in the mechanism of pit formation, so that pits are prevented even though one of the other factors, such as inorganic foreign particles transferred from 90 the anode, may still be present.

The addition of even small amounts of hydrogen peroxide to the nickel bath produces highly satisfactory results. I find that it is generally not necessary to use more than about 4 cc. of a 3% solution of hydrogen peroxide per litre of bath for each twenty-four hour run, provided the bath is initially free from organic matter or has been freed from such matter by the preliminary treatment described above. For the purpose of providing the required amount of hydrogen peroxide, I prefer to add about 4 cc. per litre to the bath upon the commencement of deposition, after 100 which the bath may be fed at intervals with the calculated amount of hydrogen peroxide solution. Since, however, nickel baths are preferably run at elevated temperatures and are therefore preferably fed with distilled water, either through an automatic feed or by the "drip system", I prefer to add the peroxide at intervals to the feed water. For this purpose I may add 4 cc. of a 3% solution of hydrogen peroxide per litre of bath 110 to that amount of feed water which the bath takes for twenty-four hours.

The effect of even this small amount of peroxide in absorbing hydrogen so as to prevent pit formation is so great that the bath 115 not only produces annealable and pitless metal with anodes which are much poorer than it is possible to otherwise use successfully, but also produces ductile metal which 120 is both pitless and annealable with a free 125

acid concentration in the bath far higher than it has been hitherto deemed possible to electrodeposit any kind of nickel out of.

However, I prefer to use my new anode referred to above, since it acts to transfer less foreign particles to the cathode than other anodes known to me, and for the further reason that such an anode maintains the metal concentration of the bath better than the other anodes customarily used. I also prefer to regulate the acidity of the bath so that the latter is only very slightly acid or even nearly neutral, thus avoiding excessive generation of hydrogen and correspondingly excessive consumption of the hydrogen peroxide, with consequently greater likelihood of forming pits and unannealable metal. While I may also add colloidal nickel hydrate to the bath containing the peroxide, I find that this is no longer necessary and that any considerable quantity of such hydrate, particularly if the bath is heated over 40° C., may cause difficulties through reacting with the peroxide and decomposing the same faster than is desirable, as well as by itself becoming oxidized or otherwise decomposed and settling out of the bath as a sludge which may act to roughen the cathode deposit. Similarly, I may provide sodium or other alkali sulphate in the bath, this material, in the form of the invention described above, being already present in the bath, due to the reaction between caustic soda and the sulphuric acid sulphates, particularly ferrous sulphate, present in the nickel salts of which the bath is prepared.

By means of the above described embodiment of my present process I am enabled to produce a ductile "nickel metal" which is not only softer than any new metal hitherto known to me, but it is also at the same time pitless and perfectly annealable. By the term "annealable" I mean that the "nickel metal" made in accordance with the present invention and whether or not it has previously had mechanical work performed upon it, may be heated to a red heat and cooled either slowly or quickly without embrittlement. Moreover if such metal has been annealed after it has been cold-worked, it will be softer than before. To illustrate the ductility of this new nickel metal, I have drawn a strip one-sixteenth of an inch square, which has been sawed from a cathode, into a wire .002 of an inch in diameter without annealing, during which operation the strip was elongated from eight inches to a length of eight hundred and thirty feet. This metal also has the unusual property of retaining, upon cold-working, considerable elongation power, while acquiring at the same time a high degree of hardness as determined by the "Brinell" test. The Brinell factor of hardness of the deposited metal will vary from about 63 to about 80, accord-

ing to conditions, and the elongation factor of such metal is approximately 32%. Upon cold-working the deposited metal to the extent indicated in the example of wire drawing given above, the Brinell factor of hardness increases to about 183, and the tensile strength of the metal has correspondingly risen from 72,000 lbs. per square inch to 250,000 lbs. per square inch, while the cold-worked metal still retains an elongation factor of 10%.

The present process has the further advantage that it avoids the necessity of the exactitude of control of the various factors of deposition, such as "pH" concentration, temperature, the current density, anode-cathode surface ratio, etc., formerly deemed necessary for the production of perfect metal. The present process is therefore cheaper to operate, particularly on a large scale.

It is of course to be understood that my invention is not limited to the particular embodiments thereof herein described for purposes of illustration only.

What I claim is:

1. The method of electrodepositing "nickel metals" which comprises treating the electrodeposition bath with chlorine to oxidize organic matter present in the bath.
2. The method of electrodepositing "nickel metals" which comprises treating the electrodeposition bath with an alkali hydrate to effect a removal of a part at least of the iron salts in solution in the bath.
3. The method of electrodepositing "nickel metals" which comprises treating the electrodeposition bath with chlorine in the presence of a metallic reducing agent to effect a removal of a part at least of the copper in solution in the bath.
4. The method of electrodepositing "nickel metals" which comprises treating the electrodeposition bath with chlorine in the presence of a metallic reducing agent under alkaline conditions to effect a removal of a part at least of the copper in solution in the bath.
5. The method of electrodepositing "nickel metals" which comprises giving the electrodeposition bath an oxidizing treatment to oxidize organic matter present in the bath, and thereafter conducting the electrodeposition in the presence of an oxidizing agent.
6. The method of electrodepositing "nickel metals" which comprises treating the electrodeposition bath with chlorine to oxidize organic matter present in the bath, and thereafter adding hydrogen peroxide to the bath.
7. The method of electrodepositing "nickel metals" which comprises treating the electrodeposition bath with chlorine in the presence of a metallic reducing agent

to effect a removal of a part at least of the copper in solution in the bath, and thereafter adding hydrogen peroxide to the bath.

8. The method of electrodepositing "nickel metals" which comprises treating the electrodeposition bath with chlorine in the presence of a metallic reducing agent under alkaline conditions to effect a removal of a part at least of the copper in solution in the bath, and thereafter adding hydrogen peroxide to the bath.

9. The method of electrodepositing "nickel metals" which comprises treating the electrodeposition bath with an alkali hydrate to remove a part at least of the iron salts in solution in the bath, and thereafter treating the bath with chlorine to effect a removal of a part at least of the copper salts in solution in the bath, and thereafter adding hydrogen peroxide to the bath.

10. A "nickel metal" electrodeposition bath containing an oxidizing agent adapted to act as a hydrogen depolarizer.

11. A "nickel metal" electrodeposition bath containing hydrogen peroxide.

12. The method of electrodepositing "nickel metals" from a bath containing iron and copper salts in solution, which comprises removing the iron and copper salts from the solution and thereafter electrodepositing "nickel metal" in the presence of an oxidizing agent while regulating the acidity of the bath whereby the deposit is rendered malleable.

13. The method of electrodepositing "nickel metals" from a bath containing iron and copper salts in solution, which comprises removing the iron and copper salts from the solution and thereafter electrodepositing "nickel metal" in the presence of hydrogen peroxide while regulating the acidity of the bath whereby the deposit is rendered pitless.

14. The method of electrodepositing "nickel metals" which comprises passing chlorine through the bath and thereafter electrodepositing "nickel metal" in the presence of an oxidizing agent while regulating the acidity of the bath so that the deposited metal is malleable.

15. The method of electrodepositing "nickel metals" which comprises passing chlorine through the bath and thereafter electrodepositing "nickel metal" in the presence of hydrogen peroxide while regulating the acidity of the bath so that the deposited metal is malleable.

In testimony whereof, I have signed my name of this specification this 31st day of July, 1921.

CHAS. P. MADSEN.